

## UNITED STATES PATENT OFFICE

2,140,367

## THERMIONIC CATHODE

Erwin F. Lowry, Wilkinsburg, Pa., assignor to  
Westinghouse Electric & Manufacturing Com-  
pany, a corporation of Pennsylvania

No Drawing. Application October 28, 1926,  
Serial No. 144,911

11 Claims. (Cl. 250—27.5)

My invention relates to thermionic cathodes and in particular to cathode materials adapted to be coated with electron-emissive oxides.

One object of my invention is to provide an inexpensive base-metal filament.

Another object of my invention is to provide a base-metal filament that will not react injuriously, at elevated temperatures, with the electron-emissive oxides carried thereby.

10 Another object of my invention is to provide a base-metal-filament material having a relatively high specific resistance.

Another object of my invention is to provide a base-metal filament that will be substantially as satisfactory in use as the platinum-iridium filaments heretofore considered necessary as carriers for oxide coatings.

Another object of my invention is to provide a method whereby my improved base-metal alloy may be prepared from the raw materials.

It has heretofore been considered necessary to employ, as a carrier for an electron emissive oxide coating, a filament made of either platinum or a platinum-iridium alloy.

25 It has been commonly accepted as a fact, among workers in the thermionic-tube art, that is to say, in the making of X-ray tubes, hot cathode rectifiers, three-electrode tubes and four electrode tubes for radio purposes and the like, that

30 metals forming acid oxides are unsuitable for this purpose. It was, consequently, deemed necessary to employ one of the so-called noble metals as a filament material, under the impression that,

35 since they were the only ones which did not react with the oxides at an elevated temperature, their use was imperative.

Among the requirements of a filament material may be mentioned freedom from oxidization at high temperatures and high specific resistances. The reason back of the first requirement is obvious. The necessity of a high specific resistance arises from the fact that the elements of substantially all thermionic tubes are relatively small in size. In order to secure the necessary

40 electron emission from a filament of perhaps only an inch in length, it is necessary that the  $I^2r$  loss be fairly large. To secure, with a limited current consumption, the necessary heating effect, it is, of course, imperative that the resistance  $r$  be large. It is also desirable that the electron-

emissive surface be fairly extensive and, since a large surface presupposes a wire having an appreciable diameter, it is obvious that the material used should have a high specific resistance.

Some of the popular high-resistance alloys 5 which are extensively used in high-temperature work, such as those known under the trade-marks Nichrome, Chromel and Karma, are of the type which form acid oxides. They have, consequently, been considered unsuitable for use as a filament material.

Other characteristics necessary in a suitable filament material are a reasonable tensile strength at 1000° C. and sufficient ductility to enable it to be drawn readily into fine wire not 15 larger than 10 mils in diameter.

No single metal, with the possible exception of platinum, and no heretofore employed alloy, except platinum-iridium, has embodied all of the necessary requirements mentioned. It is, accordingly, the principal object of my invention, as stated previously, to produce an alloy which will satisfactorily replace platinum or platinum-iridium and which will be very much cheaper to manufacture.

20 I have made numerous experiments with alloys of different metals and have discovered that metals of the iron group are the only ones, apparently, that meet all of the above requirements and I have also discovered that these metals are not 25 entirely satisfactory in a pure state.

The alloy that I have found to be the most satisfactory, comprises nickel, cobalt, iron and titanium. Varying proportions of these elements have been employed with an approximation of 30 equally good results. I have used alloys containing nickel and cobalt in the aggregate of 80 to 95%, in which the nickel and cobalt were present in proportions ranging from 95 to 5% nickel to 5 to 95% cobalt. The combination nickel-cobalt has a higher resistance and is less susceptible to chemical attack by the oxide-coating materials used than either of the metals alone. The remainder of the alloy consists of metals which render the nickel-cobalt alloy forgeable and, among other things, remove oxides from the alloy. Therefore, I introduce into the alloy from 35 5 to 20% of ferrotitanium, ferrovanadium, ferrosilicon or ferromolybdenum in an amount sufficient to render the nickel-cobalt forgeable and 40 50

ductile so that the ingot may be reduced to a fine wire or may be otherwise shaped.

One alloy in particular which I have found extremely satisfactory may be made by combining

|    |          |       |
|----|----------|-------|
| 5  |          | Parts |
|    | Nickel   | 80    |
|    | Cobalt   | 20    |
|    | Iron     | 7½    |
| 10 | Titanium | 2½    |

10 the iron and titanium being used in the form of a ferro-titanium alloy. A typical analysis of the complete alloy is as follows:

|    |          |         |
|----|----------|---------|
| 15 |          | Percent |
|    | Nickel   | 70      |
|    | Cobalt   | 19½     |
|    | Iron     | 7½      |
|    | Titanium | 2½      |

20 The process of preparing this alloy is substantially as follows:

The above-mentioned proportions of nickel, cobalt, and ferro-titanium are melted together in an electric furnace, care being taken to prevent access of oxygen. After the melt is completed and just before casting, a small amount of magnesium and aluminum is added to serve as de-oxidizing agents. There is also a possibility that the ferro-titanium functions as a 25 de-oxidizing agent as well, and it is within the scope of my invention to use ferro-titanium, ferro-vanadium, silicon, ferro-silicon, manganese or ferro-manganese.

The ingot resulting from the melt is subsequently forged at about 750° C. My experiments seem to indicate that the forging temperature has an important bearing upon the molecular structure of the finished filament, and this temperature should not be permitted to go much 35 above 800° C.

By repeated forging, the ingot is reduced to a convenient size for rolling and swaging, by which latter operation it is reduced to a diameter of about 50 mils.

45 It is imperative that, in the rolling and swaging processes, the metal shall be annealed after every second die.

The 50 mil diameter wire is then drawn down to the required size through diamond dies of 50 successively smaller diameters. It is noted that substantially no annealing is necessary after a size of 10 mils has been attained.

I have found that the finished filaments have resistances of approximately 40 ohms per mil-inch as compared with 22 ohms per mil-inch for a 10% platinum-iridium alloy. This feature is of distinct advantage because it practically doubles the cross-section of a filament having the same electrical and thermionic characteristics as 60 a filament of a given size composed of platinum-iridium.

This high specific resistance has a further advantage in that it will permit filaments of the oxide-coated type to be made having certain filament voltage-current relations which have been heretofore commercially impracticable when employing platinum-iridium. For example, a filament .75 inch long may be made from my improved nickel-cobalt alloy which will reach the 70 proper operating temperature at .3 volt and .06 ampere. This feature will enable the thoriated tungsten filament in tubes, such as the small UV-199, to be replaced by oxide-coated filaments.

75 My nickel-cobalt alloys have an extremely high tensile strength when cold, a tensile strength of

over 100,000 lbs. per sq. in. not being unusual. The utilization of a material of such strength greatly decreases the likelihood of breakage during manufacture.

Furthermore, it has been found that filaments made of certain of these nickel-cobalt alloys will have the very advantageous property that, when heated to 1000° C., they will stretch as much as 10 to 12% of their length before breaking. This stretching, when heated, obviates the necessity 10 for a critical adjustment of a spring support to prevent sag caused by thermal expansion. The "take-up" of the spring must be only slightly greater than the thermal expansion expected, and the rather critical adjustment of the filament hooks to take care of the expansion that takes place in platinum-iridium filaments is unnecessary. For this reason, a filament comprising my new alloy will be non-microphonic since it will stretch, under tension of the springs, until the tension is relieved at the operating temperature. The limits thus set for the spring "take-up" are, accordingly, not less than the thermal expansion of the filament and not more than 10% of the filament length.

I have found also that cobalt is a very satisfactory material with which to electroplate a filament, otherwise unsatisfactory, as a carrier for emissive oxides. The cobalt, in this case, serves to protect the oxide coating from the 30 harmful influence of the base-metal-filament. For this purpose, the cobalt may be applied to the filament material as a sleeve instead of by electroplating and both metals drawn down and rolled to the required size together.

No special technique is required in applying the oxide coatings to filaments of any of the herein described alloys or to filaments which have previously been coated with pure cobalt, although a mixture of the carbonates of barium 40 and strontium suspended in ethyl-alcohol is suggested as being the most satisfactory coating compound.

Where the expression "cobalt-nickel" occurs in the claims, it signifies that the proportion of cobalt to nickel lies within the limits specified previously, namely 95 to 5% nickel and 5 to 95% cobalt. Where the claims state that a core or alloy or filament comprise particular elements, it means that no other substances are present in such amount as would substantially affect the properties of the resulting material.

Although I have described herein certain specific embodiments of my invention, other modifications will be apparent to those skilled in the art. My invention, therefore, is not to be limited except insofar as is necessitated by the prior art and as indicated in the appended claims.

I claim as my invention:

1. In combination with an evacuated container, an electrode comprising a base metal composed of an alloy comprising cobalt-nickel and titanium and a layer of electron-emissive material on said base metal, said cobalt nickel being from 80 per cent to 95 percent of said alloy.

2. In combination with an evacuated container, an electrode comprising a base metal composed of an alloy consisting of a compound of cobalt and nickel of which neither constituent is less than 5% and an element of the group consisting of titanium, vanadium and manganese, and a layer of electron-emissive material on said base metal, said compound being from 80 percent to 95 percent of said alloy.

3. A cathode element for an electron dis-

charge device composed of an alloy comprising a base selected from the group comprising nickel and cobalt and constituting at least 90% of the alloy, and an added quantity of substance taken 5 from the group comprising silicon, titanium, vanadium and zirconium, the added quantity including at least silicon and titanium, the silicon constituting at least  $\frac{1}{2}$  of 1% of the alloy, and the titanium constituting at least  $\frac{1}{4}$  of 1% of the alloy.

4. A cathode element for an electron discharge device composed of an alloy comprising a base selected from the group comprising nickel and cobalt and constituting at least 90% of the alloy, 10 and an added quantity of substance taken from the group including silicon, titanium, vanadium and zirconium, the added quantity including at least silicon and vanadium, the silicon constituting at least  $\frac{1}{2}$  of 1% of the alloy, and vanadium 15 constituting at least  $\frac{1}{4}$  of 1% of the alloy.

5. In a hermetically sealed evacuated tube, a metallic cathode element exposed to the rarefied atmosphere within said tube and composed of a malleable and ductile deoxidized and degasified 20 alloy comprising a metal having the characteristics common to nickel and cobalt and containing silicon, and low in carbon.

6. In a hermetically sealed evacuated tube, a metallic cathode element exposed to the rarefied atmosphere within said tube and composed of a malleable and ductile alloy comprising a metal having the characteristics common to nickel and cobalt and containing a deoxidizer in excess of the amount required to effect substantial deoxidation 25 so as to effect also substantial degasification of the alloy, the unoxidized excess remaining in the alloy as a constituent thereof, said alloy being low in carbon.

7. In a hermetically sealed evacuated tube, a 40 metallic cathode element exposed to the rarefied

atmosphere within said tube and composed of a malleable and ductile alloy comprising a metal having the characteristics common to nickel and cobalt and containing silicon in excess of the amount required to effect substantial deoxidation so as to effect also substantial degasification of the alloy, the unoxidized excess of the silicon remaining in the alloy as a constituent thereof, said alloy being low in carbon. 5

8. In combination with an evacuated container, an electron-emissive cathode having a core comprising cobalt, nickel, titanium and iron, said cobalt and nickel being from 80% to 95% and said titanium and iron being from 5% to 20% of said core. 10

9. In combination with an evacuated container, an electrode comprising a base metal composed of an alloy comprising cobalt, nickel, iron and titanium and a layer of electron-emissive material on said base metal, said cobalt and nickel 15 being from 80% to 95% and said iron and titanium being from 5 to 20% of said alloy. 20

10. In combination with an evacuated container, an electrode comprising a base metal composed of an alloy comprising cobalt, nickel and iron and an element of the group consisting of titanium, vanadium and manganese, and a layer of electron-emissive material on said base metal, said cobalt and nickel being from 80% to 95% 25 of said alloy and said iron and element being 30 from 5% to 20% of said alloy.

11. A cathode comprising a base metal consisting of 80% to 95% of a compound of cobalt and nickel of which neither constituent is less than 5% and the remaining 20% to 5% a deoxidizer consisting of one or more of the metals iron, 35 titanium, vanadium or silicon and an electron-emissive coating on said base metal.

ERWIN F. LOWRY. 40